

## UNITED STATES PATENT OFFICE

2,182,140

## PROCESS FOR PRODUCING RESERVES UNDER DYEINGS OF ESTER SALTS OF LEUCO VAT DYESTUFFS

Ernst Tschan, Basel, Switzerland, assignor to the firm Durand &amp; Huguenin A. G., Basel, Switzerland

No Drawing. Application March 20, 1935, Serial No. 12,106. In Germany March 26, 1934

## 4 Claims. (Cl. 8—65)

The sunnuric acid esters of leuco vat-dyestuffs, respectively their salts (ester salts), see United States Patent No. 1,448,251, regenerate by means of acid oxidation the original vat-dyestuff (for instance on the fibre) and allow to produce by this way dyeings and prints which, on account of their perfect levelness and penetration as well as good fastness properties, find a great success amongst dyers and printers.

These ester salts also allow the fabrication of fancy figured dyeings, a result which could scarcely be obtained by hitherto usual means.

It is therefore possible to produce, for instance on a ground dyed with an ester salt, white and colored reserves. Similar methods are described in the United States Patent 1,575,958. This process consists in printing either on the white material or on a fabric padded in a bath containing a solution of an ester salt and afterwards 20 dried, a reserve paste containing either a body of alkaline reaction or a reducing agent, or both together. On the printed places the development by acid oxidation of the ester salt dyeings does not take place as the action of acid and 25 oxidizing agent is rendered impossible. In this manner white reserves on a colored ground can be obtained. By adding vat-dyestuffs to the reserve paste colored reserves may also be obtained.

There are, however, ester salts which according to this process can only be reserved with difficulty and which are not suitable for this purpose. This drawback may have two reasons: Certain ester salts have such a pronounced affinity to the cotton fibre that it is no more possible 30 either by washing at the boil or by soaping to remove the unoxidized ester salt off the fibre. Some ester salts are easily oxidizable respectively very sensitive to acid. The alkali and the reducing agent of the reserve paste are not sufficient 35 to protect the ester salt against saponification and oxidation. It is a fact that in many cases, not in all, these two drawbacks, which prevent the production of good reserve effects 40 are particular to the same ester salt. This is 45 increasing the difficulties.

Amongst the hardly reserveable ester salts, some give dyeings and prints of especially good fastness and can therefore not be replaced by 50 other ester salts.

Green dyeings made of the ester salt of the leuco dimethoxy-dibenzanthrone can, for instance, not be reserved; the affinity thereof to the fibre is so great that this ester salt remains 55 on the latter as a red body. The discharging of

such a dyeing is also not practicable for the same reason.

Some dyeings obtained from the leuco dibromo-dibenzpyrenequinone respectively from the leuco di-benzpyrenequinone are also for the reason of their affinity only reserveable or dischargeable in light shades.

It has now been found that according to the process of this invention it is possible to produce good reserves under ester-salt dyeings, also under dyeings of such ester salts which could not be reserved in satisfactory manner by the hitherto employed processes. According to this invention, on the white material, before padding, a reserve paste is printed containing—besides an alkali, especially an alkaline carbonate—a quaternary ammonium compound, i. e., a compound in which four valences of the nitrogen atom are substituted by organic radicals. One pads afterwards as usual in a solution of an ester salt, dries 20 and develops the shade, according to the known working methods, by treating with an oxidizing agent in the presence of acid. The methyl-sulphuric salt of trimethylphenyl-ammonium hydroxide, the dimethylphenylbenzyl-ammonium 25 chloride, the benzylpyridinium chloride, the methylpyridinium chloride respectively the corresponding free bases and others are suitable for the present purpose. The insolubility of these bodies prevents them from penetrating into the fibre. Their oxidation to the dyestuff takes place outside the textile material, so that by a soaping 30 at the boil they can be removed, whereby pure white reserves are resulting.

The production of a pure white is also improved 35 by a treatment in an acid bath. It is therefore recommended, when applying for instance the steam process, in which the development is carried out by steaming, to pass the material for a short time in an acid bath after the development. When applying the other processes (nitrite-bichromate-chromate), the treatment for developing the shade by means of an acid bath is already fulfilled. The sodium carbonate contained in the reserve paste is decomposed on the fibre by the acid of the bath and gaseous carbonic acid is formed. This latter removes the insoluble compound of the ester salts and the quaternary ammonium off the fibre and facilitates in this way the reserving.

This new process allows the production of a new interesting style, which could not hitherto be executed. This special style is only obtainable with ester salts of leuco vat-dyestuffs, but it can 55

not be realized by means of the vat-dyestuffs themselves.

The following examples illustrate the present invention.

5

*Example 1*

On white material there is printed the following reserve color:

|                               | Gr.  |
|-------------------------------|------|
| 10 Anhydrous sodium carbonate | 150  |
| Water                         | 300  |
| Gum thickening (1:1)          | 500  |
| Benzylphenylammonium chloride | 50   |
|                               | 1000 |

15

Then the material is dried and padded in a full bath containing the following solution:

|                                                          | Gr. |
|----------------------------------------------------------|-----|
| 20 Ester salt of leuco dimethoxydibenzanthrone 20% paste | 80  |
| Water                                                    | 500 |
| Neutral tragacanth thickening                            | 50  |
| Solution of sodium carbonate (10%)                       | 20  |
| 25 Solution of sodium nitrite (20%)                      | 50  |

the whole being brought with water to 1 liter.

The material is then dried, passed for about 3-5 seconds in a bath at 60° C. containing 36 gr. of concentrated sulphuric acid per liter, washed, 30 soaped at the boil, rinsed and again dried.

By this way white reserves on green ground are obtained.

It is possible to replace the ester salt of the leuco-dimethoxydibenzanthrone by the ester salt 35 of leuco-dibenzpyrene-quinone or leuco-dibromodibenzpyrene-quinone as well as by the ester salt of the tetrahydrodianthraquinoneazine. There are accordingly obtained white reserved effects on yellow or blue ground respectively.

40

*Example 2*

On white material there is printed the following reserve color:

|                                                            | Gr.  |
|------------------------------------------------------------|------|
| 45 Anhydrous sodium carbonate                              | 150  |
| Water                                                      | 300  |
| Methyl-sulphuric salt of trimethylphenylammonium hydroxide | 50   |
| Gum thickening (1:1)                                       | 500  |
|                                                            | 1000 |

50

The material is dried and passed in a full bath containing the following solution:

|                                                                                                          | Gr. |
|----------------------------------------------------------------------------------------------------------|-----|
| 55 Ester salt of the known leuco vat-dyestuff according to Example 1 of German Specification No. 212,471 | 20  |
| Water                                                                                                    | 500 |
| Solution of sodium carbonate (10%)                                                                       | 20  |
| 60 Gum tragacanth thickening                                                                             | 50  |
| Solution of sodium nitrite (20%)                                                                         | 50  |

the whole being brought with water to 1 liter.

This is then dried and developed as given in 65 Example 1. Pure white effects on olive ground are obtained.

*Example 3*

On white material there is printed a reserve color made of:

|                              | Gr. |
|------------------------------|-----|
| Sodium carbonate             | 150 |
| Water                        | 270 |
| Gum thickening (1:1)         | 500 |
| 75 Benzylpyridinium chloride | 80  |

This is then dried and padded in a full bath containing the following solution:

|                                                 | Gr. |
|-------------------------------------------------|-----|
| Ester salt of dimethoxydibenzanthrone 20% paste | 80  |
| Ethylene-thioglycol                             | 50  |
| Water                                           | 500 |
| Tragacanth thickening (60%)                     | 50  |
| Solution of sodium chlorate (10%)               | 120 |
| Sulphocyanide of ammonia (1:1)                  | 60  |
| Solution of vanadate of ammonia (1%)            | 10  |
| Aqueous solution of ammonia (25%)               | 10  |

the whole being brought with water to 1 liter.

Thereupon, it is dried, steamed for 8 minutes, passed in the open-width for a few seconds in a bath containing 18 gr. of concentrated sulphuric acid per liter, at a temperature of 50° C., rinsed, soaped at the boil, rinsed again and dried.

The described process may be combined with the well known process for producing dyeings with the aid of ice color preparations which are developable by an acid treatment. Therefore, colored reserve effects may be produced by adding to the described reserve paste an ice color preparation. The fabric is printed therewith and dried and then, in well known manner, steamed under acid conditions in order to develop the ice color dyeing. The subsequent padding of the so prepared material with a solution of an ester salt of a leuco vat-dyestuff, further the development of the ester-salt-dyeing is principally the same as described.

This modification of the process is illustrated by the following examples, the parts being by weight.

*Example 4*

The following reserve color is prepared:

|                                                                                                                                                    | Parts |
|----------------------------------------------------------------------------------------------------------------------------------------------------|-------|
| An ice color preparation containing a diazo-amino compound of 4-nitro-2-aminoanisole and 2-hydroxy-3-naphthoyl-p-anisidide, in the commercial form | 40    |
| Caustic soda lye 38° Bé                                                                                                                            | 80    |
| Alcohol                                                                                                                                            | 30    |
| Water                                                                                                                                              | 45    |
| Gum                                                                                                                                                | 130   |
| Zinc oxide paste (1:1)                                                                                                                             | 500   |
| Methyl-sulphuric salt of trimethylphenylammonium chloride                                                                                          | 200   |
|                                                                                                                                                    | 50    |
|                                                                                                                                                    | 30    |
|                                                                                                                                                    | 1000  |

After printing this is dried and aged for 4 minutes, while spraying a mixture of acetic acid and formic acid (equal parts) into the apparatus to bring the steam to acid reaction to litmus paper. Then there is padded in the following padding bath:

|                                                       | Parts |
|-------------------------------------------------------|-------|
| Ester salt of leuco-dimethoxydibenzanthrone 20% paste | 50    |
| Water                                                 | 500   |
| Tragacanth thickening                                 | 50    |
| Sodium carbonate                                      | 2     |
| Sodium nitrite                                        | 15    |

the whole being brought to one liter.

After padding it is dried and treated for 8 minutes at 60-70° C. in a bath containing 36 gr. of concentrated sulphuric acid per liter. Then it is rinsed, neutralized with some sodium carbonate and soaped at the boil. Thus bright red reserves on green ground are obtained.

75

## Example 5

The following reserve color is printed on white material:

|                                                                                                                                            | Parts |
|--------------------------------------------------------------------------------------------------------------------------------------------|-------|
| 5 Ice color preparation containing a diazo amino compound of metantraniline and 2-hydroxy-3-naphthoyl-anilide in the usual commercial form | 80    |
| 10 Alcohol                                                                                                                                 | 30    |
| Water                                                                                                                                      | 160   |
| Gum                                                                                                                                        | 500   |
| Zinc oxide paste (1:1)                                                                                                                     | 200   |
| Methyl-sulphuric salt of trimethylphenyl-ammonium chloride                                                                                 | 30    |
| 15                                                                                                                                         | 1000  |

This is then dried and steamed as given in Example 4 for a few minutes in acid steam, and then padded in the following padding bath:

|                                                       | Parts |
|-------------------------------------------------------|-------|
| Ester salt of leuco-dimethoxydibenzanthrone 20% paste | 50    |
| 25 Water                                              | 500   |
| Tragacanth thickening                                 | 50    |
| Solution of sodium chlorate (10%)                     | 80    |
| Sulphocyanide of ammonia (1:1)                        | 40    |
| Solution of vanadate of ammonia (1%)                  | 10    |
| 30 Aqueous ammonia (20%)                              | 20    |

the whole being brought with water to one liter.

It is then dried, steamed for 8 minutes and thereupon treated in a bath containing 36 gr. of concentrated sulphuric acid per liter. To finish it is soaped, neutralized with some soda and soaped at the boil.

Bright orange reserves on green ground are thus obtained.

## Example 6

The following reserve color is prepared:

|                                                                                                                                            | Parts |
|--------------------------------------------------------------------------------------------------------------------------------------------|-------|
| 45 Ice color preparation containing diazo amino compound of ortho-chloraniline and di-aceto-acetic-o-tolidide in the usual commercial form | 80    |
| Caustic soda (38° Bé.)                                                                                                                     | 30    |
| 50 Alcohol                                                                                                                                 | 30    |
| Water                                                                                                                                      | 130   |
| Gum                                                                                                                                        | 500   |
| Zinc oxide paste (1:1)                                                                                                                     | 200   |
| Methyl-sulphuric salt of the trimethyl-phenylammonium chloride                                                                             | 30    |
| 55                                                                                                                                         | 1000  |

This is printed on white material, dried, steamed as given in Example 4 and padded in a padding bath containing:

|                                                                                                     | Parts |
|-----------------------------------------------------------------------------------------------------|-------|
| Ester salt of the leuco vat-dyestuff as per Example 4 of German Specification No. 212,471 20% paste | 60    |
| 65 Hot water                                                                                        | 500   |
| Tragacanth thickening                                                                               | 50    |
| Sodium carbonate                                                                                    | 2     |
| Sodium nitrite                                                                                      | 20    |

70 the whole being brought with water to one liter. Then it is dried as given in Example 4, developed in an acid bath, rinsed and soaped. Yellow reserve effects on olive ground are obtained.

## Example 7

The following reserve color is prepared:

|                                                                                                                                                     | Parts |
|-----------------------------------------------------------------------------------------------------------------------------------------------------|-------|
| Ice color preparation containing the nitro-amine of diazotized meta-nitra-para-toluidine and 2-hydroxy-3-naphthoyl-anilide in usual commercial form | 5     |
| Ammonium salt of ricinol sulphuric acid                                                                                                             | 100   |
| Water                                                                                                                                               | 40    |
| Caustic soda lye (38° Bé.)                                                                                                                          | 194   |
| Gum                                                                                                                                                 | 16    |
| Methyl-sulphuric salt of the trimethyl-phenylammonium chloride                                                                                      | 10    |
| Zinc oxide paste (1:1)                                                                                                                              | 400   |
|                                                                                                                                                     | 200   |
|                                                                                                                                                     | 15    |
|                                                                                                                                                     | 1000  |

This is then printed on white material, dried aged for 4 minutes as described in Example 4 in acid conditions. Afterwards it is padded in a padding solution of the same composition as in Example 4 and developed in an acid bath. Finishing takes place as already described.

Red reserve effects on green ground are obtained.

Instead of the methyl-sulphuric salt of trimethylphenylammonium chloride, one can use with similar result another quaternary ammonium compound, for example one of those mentioned in the introduction of this specification.

What I claim is:

1. In the process of producing reserve effects under dyeings obtained with the aid of ester salts of leuco vat dyestuffs, the step which comprises producing upon the textile material local resists against the ester salts by applying to said material locally an alkaline printing paste containing a thickening agent and a water-soluble compound of the general formula



40

wherein  $\text{R}_1$ ,  $\text{R}_2$ ,  $\text{R}_3$  and  $\text{R}_4$  designate alkyl, aralkyl or aryl radicals having no sulpho or carboxy substituents, while  $\text{X}$  stands for the anion of a water-soluble salt.

2. In the process of producing reserve effects under dyeings obtained with the aid of ester salts of leuco vat dyestuffs, the step which comprises producing upon the textile material local resists against the ester salts by applying to said material locally an alkaline printing paste containing a thickening agent and dimethyl-benzyl-phenyl-ammoniumchloride.

3. In the process of producing reserve effects under dyeings obtained with the aid of ester salts of leuco vat dyestuffs, the step which comprises resisting local areas of the textile material against the action of said dyestuffs by applying to the fabric, prior to the coloring treatment, a resist paste comprising a water-soluble salt of a quaternary ammonium compound, a thickening agent and an alkaline agent of the type commonly employed in printing with vat dyestuffs.

4. A process for producing white reserve effects under dyeings obtained with the aid of ester salts of leuco vat dyestuffs, consisting in applying to the fabric an alkaline reserve paste containing anhydrous sodium carbonate, gum thickening and dimethyl-benzyl-phenyl-ammoniumchloride, drying, further padding with a solution of the ester salt of leuco dimethoxydibenz-anthrone and finally developing the dyeing by acid oxidation.

ERNST TSCHAN. 76